# EUROPEAN PATENT SPECIFICATION

(11) **EP 0 064 877 B1**
(45) Date of publication and mention of the grant of the patent: **15.01.1986**
(21) Application number: 82302373.4
(22) Date of filing: 10.05.1982
(51) Int. Cl.: C22B 60/02, C01G 43/00

(54) **A liquid membrane process for uranium recovery**
Flüssig-Membran-Verfahren zur Gewinnung von Uran
Procédé avec membranes liquides pour la récupération de l'uranium

(30) Priority: 11.05.1981 US 262394
(43) Date of publication of application: 17.11.1982
(73) Proprietor: EXXON RESEARCH AND ENGINEERING COMPANY, Florham Park, New Jersey 07932-0390 (US)
(72) Inventor: Cahn, Robert Paul, Millburn New Jersey (US); Valint, Paul Louis, Jr., Rahway New Jersey (US)
(74) Representative: Field, Roger Norton (GB)

## Description

This invention relates to a process for recovering uranium from aqueous solution. More particularly, this process relates to an improved emulsion extraction process for recovering uranium from a WPPA feed solution which comprises adding excess oxidizing agent to the feed. Still more particularly, this invention relates to an improved process for recovering uranium from a WPPA feed solution containing uranyl cations which comprises adding excess oxidizing agent to the feed before or while it is contacted with the emulsion extractant.

Recovering uranium as a by-product from wet process phosphoric acid is well-known in the art. Phosphate rock is mined primarily to produce a high-phosphate containing fertilizer, the first step of which involves digesting the rock in sulfuric acid to produce a phosphoric acid solution which is known in the art as wet process phosphoric acid (WPPA). This WPPA contains uranium which can be recovered before the acid is further processed for making fertilizer. This uranium is present in the acid primarily as UOl+ cations referred to in the art as uranyl ions, wherein the uranium is in the hexavalent, +6 state. In known processes for recovering uranium from WPPA, the uranium is extracted from the WPPA by contacting the WPPA with an extractant which is an oily, water-immiscible material consisting of a mixture of di-2-ethylhexyl phosphoric acid (D2EHPA) and trioctylphosphine oxide (TOPO) dissolved in an oily, organic liquid such as' kerosene. The amount of uranium that the oily extractant can contain is limited by equilibrium conditions. This is quite low and is generally less than one gram of uranium per liter of extractant. The uranium enriched extractant is then separated from the WPPA and contacted with an aqueous solution containing a reducing agent such as ferrous ions in an acid such as phosphoric acid, to convert the uranium to tetravalent U(IV) ions. The U(IV) ions are relatively insoluble in and are not re-extracted by the D2EHPA/TOPO-containing oil. This step results in stripping the uranium from the oily extractant into the aqueous reducing solution and the aqueous reducing solution is then further processed to recover the uranium. Thus, at least two different extraction operations are required. Typical of the prior art which teaches the recovery of uranium from WPPA by first contacting the acid with an oily extractant containing D2EHPA/TOPO, separating the uranium-enriched extractant from the uranium-reduced feed and then stripping the uranium from the uranium-enriched extractant with an aqueous reducing solution of ferrous ions in phosphoric acid are U.S. Patents 3,711,591 and 3,737,513.

Unfortunately, this well-known and commercially practised process for recovering uranium from WPPA suffers from many disadvantages, among which is a relatively low extraction efficiency ranging from about 1 to about 7. Extraction efficiency is defined as the ratio of the uranium concentration in the oily extractant to the uranium concentration remaining in the WPPA feed at extraction equilibrium conditions. Low extraction efficiency means that large quantities of expensive D2EHPA/TOPO extractant must be used and circulated with high concomitant losses of expensive reagents. Additionally large, expensive contacting vessels and settling tanks and pumps are required to handle large amounts of oily extractant. Another drawback of this process is due to the fact that as the temperature increases, the extraction efficiency decreases. For example, a report issued by the Oak Ridge National Laboratories (cf. Solvent Extraction of Uranium from Wet Process Phosphoric Acid, F. J. Hurst, D. J. Crouse and K. B. Brown, Report from Oak Ridge National Laboratory, April, 1969) disclosed that the extraction efficiency decreased from about 7 to about 1 when the extraction temperature, increased only from about 20°C to 60°C when uranium was extracted from WPPA using a solution of 0.2M D2EHPA and 0.5M TOPO in kerosene as the extractant. At a temperature of 40°C the extraction efficiency was 2. As a consequence, commercial processes must either operate at a temperature no higher than about 40°C or include more extraction stages to maintain a higher efficiency at the higher temperatures. The WPPA is produced at a temperature of about 60°C which means that the acid must be cooled down to about 40°C before being extracted or additional extraction stages must be used to maintain satisfactory extraction efficiency at the higher temperature. This naturally necessitates additional equipment and the use of considerable amounts of energy to cool the WPPA down to an economically viable extraction temperature.

It is known to use an emulsion process for recovering uranium from uranium-bearing WPPA streams. This emulsion process comprises contacting a uranium containing WPPA feed with globules of a water-in-oil emulsion comprising microdroplets of an aqueous interior phase dispersed in an oily, continuous exterior phase containing at least one transfer agent for selectively transferring the uranium from the feed into the interior phase of the emulsion wherein the valence of the uranium species is changed, thereby trapping the uranium in the emulsion. The uranium-enriched emulsion is then separated from the feed, the emulsion is broken and the uranium is recovered.

In a preferred embodiment of this process, the uranium is present in the WPPA feed as uranyl ion, the exterior phase contains a mixture of D2EHPA and TOPO as selective transfer agents for the uranyl ion and the interior phase of the emulsion contains a reducing agent which changes the uranyl to U(IV) ions, thereby trapping the uranium in the interior phase of the emulsion as uranous ions.

It has now been discovered that the liquid membrane emulsion extraction process known in the art is improved if excess oxidizing agent is added to the uranyl ion-containing WPPA feed before and/or while the feed is contacted with the emulsion. By excess oxidizing agent is meant oxidizing agent in an amount greater than that initially added to the WPPA feed, if necessary, in order to ensure that all of the uranium in said feed is in the uranyl or hexavalent form and that any iron in the feed is in the ferric or trivalent form.

It is known in the art (FR-A-2374931) to initially oxidize or add oxidizing agent to the WPPA feed in order to ensure that all of the uranium is present therein as uranyl cations before contacting the feed with an extracting agent. In the liquid membrane extraction process, we have discovered that by adding to the feed excess oxidizing agent or oxidizing agent beyond that needed to initially ensure that the uranium in the feed is in the hexavalent state, one will obtain greater levels of uranium extraction and achieve higher levels of extracted uranium in the emulsion. Thus, this invention is an improvement in an emulsion process for recovering uranium from a WPPA feed solution wherein the uranium ions initially are oxidised by adding an oxidising agent to said feed solution in order to ensure that all uranium is present in the hexavalent form, said process comprising (a) contacting, preferably, at a temperature of from about 30 to 100°C, said WPPA feed with a water-in-oil emulsion comprising (i) an aqueous interior phase dispersed in (ii) an oily exterior phase immiscible with both said interior phase and said WPPA feed solution, said interior phase comprising an acid solution containing a reducing agent and said exterior phase comprising a surfactant-containing hydrocarbon solution of D2EHPA and TOPO which transfer the uranyl ion from the WPPA solution to interior phase of the emulsion wherein said uranyl ion is reduced to the tetravalent U(IV) ion to form a uranium-rich emulsion, (b) separating the uranium-rich emulsion from the WPPA solution, and (c) recovering the uranium from the emulsion, wherein the improvement comprises adding oxidant to the WPPA feed before and/or during contacting the WPPA with the emulsion in a quantity in excess of that needed to ensure initially that the uranium in the feed is in the hexavalent state and in a quantity to ensure that any iron in the feed is in the trivalent state. In a preferred embodiment the contacting will take place in a plurality of zones.

The total amount of excess oxidant to be added will, of course depend on the feed and emulsion compositions and also on the process conditions. In general, the minimum amount of excess oxidant added to the feed will be that amount just in excess of that stoichiometrically needed to oxidize any U(IV) and ferrous ions that transfer back to the WPPA feed (due to leakage and/or breakage of the emulsion) to uranyl and ferric ions, respectively. The so-formed uranyl ions are then reextracted by the emulsion. The exact amount of excess oxidizing agent used will, of course, depend on both the amount of U(IV) and ferrous ion going back into the feed and the amount of uranium it is desired to extract from the WPPA. Any suitable oxidizing agents may be used in the process of this invention. Illustrative, but non-limiting examples of suitable oxidizing agents include chlorates, persulfates and peroxides such as hydrogen peroxide.

Contacting of the WPPA feed and emulsion is generally done in a countercurrent manner in a plurality of stages, each stage comprising at least one mixing zone and a settling zone, the mixing zone containing suitable means for mixing the WPPA feed with the emulsion. Illustrative, but non-limiting examples of suitable mixing means includes turbine and propeller mixers, static mixers, wire mesh, ultrasonic vibrations, etc. It is well-known that countercurrent extraction in a plurality of stages results in better extraction efficiency and requires less extracting agent or emulsion than a single.stage. It is preferred that each stage contains a plurality of co-current mixing zones or compartments. Employing a plurality of smaller mixing zones in each stage as opposed to a lesser number of larger zones enables one to minimize the size of mixing equipment required to achieve a given amount of extraction as those skilled in the art will know based on the well known continuous-stirred-transfer-reactor (CSTR) theory.

When the feed and emulsion are contacted in a mixing zone, a small amount of internal aqueous phase of the emulsion leaks into the feed due to minor breakage of the emulsion from the mixing shear and rupture caused by internal phase swelling. Internal phase swelling is an osmotic effect resulting from difference in ion strength across the hydrocarbon membrane of the emulsion. Since the internal aqueous phase of the emulsion contains both extracted uranium in. the tetravalent form and ferrous ion reducing agent, this leakage reduces the overall efficiency of the process by putting uranium back into the feed and by introducing iron into the feed which later requires that more oxidant be used to maintain the uranium in the feed in the hexavalent (uranyl) form.

In a preferred embodiment of this invention, the interior phase of the emulsion will be a phosphoric acid solution containing ferrous ions and the oily, water and feed-immiscible exterior phase of the emulsion will be a mixture of D2EHPA/TOPO in an aliphatic hydrocarbon which also contains a surfactant for forming and stabilizing the emulsion. The D2EHPA/TOPO in the exterior phase transports the U022+ cations from the WPPA feed into the interior phase of the emulsion wherein the uranium is stripped from the D2EHPA/TOPO by the phosphoric acid and reduced to U(IV) ions by the ferrous ions and is thereby trapped in the emulsion.

Essential to the successful operation of the process of this invention is a suitable water-in-oil type of emulsion. It has been discovered that emulsions of the type disclosed in U.S. 3,779,907, are suitable for use in the process of this invention. These emulsions are referred to liquids include substantially aliphatic hydrocarbons such as kerosene and paraffinic hydrocarbons such as Norpar 13, SK-100, Low Odor Paraffin Solvent (LOPS) and Solvent Neutral 100 (S-100N), which are available from Exxon Chemical Company. ("Norpar" and "Exxon" are registered Trade Marks, at least in the United Kingdom). It is understood, of course, that the hydrocarbon may contain one or more other hydrocarbons, halogenated hydrocarbons or higher oxygenated compounds such as alcohols, ketones, acids or esters as long as the emulsion is stable and the exterior phase is immiscible with both the aqueous feed solution and aqueous interior phase and permits transferring the uranium from the feed to the interior phase of the emulsion. The exterior phase of the emulsion will contain from about 60-98 weight % of this hydrocarbon liquid, preferably from about 75-95% and most preferably from about 85-95 weight %.

As hereinbefore stated, the oily, water immiscible external phase of the emulsion will contain one or more oil soluble surfactants for forming and stabilizing the emulsion, but which will not prohibit transfer of the uranium through the exterior phase to the interior phase. Suitable surfactants may be selected from among oil soluble anionic, cationic, and nonionic surfactants. Surfactants that have been found to be particularly suitable for use in the process of this invention include various derivatives of polyisobutylene succinic anhydride (PIBSA) which includes, but is not limited to polyamine derivatives thereof for example those having the general formula: wherein
R₁, R₂, R₃, R₄, R₅, R_{«}, and R, and Y are hydrogen, C, to C₂₀ alkyl, C₆ to C₂₀ aryl, C₇ to C₂₀ alkaryl radicals or substituted derivatives thereof; and x is an integer of from 1 to 100. R₃, R₄, R₅, R₆ and R₇ are preferably hydrogen, with x preferably varying from 3 to 20. The substituted derivatives are preferably oxygen, nitrogen, sulfur, phosphorus and halogen-containing derivatives. Various PIBSA-polyamine compounds that have been found useful in the practice of this invention include those taught in U.S. Patent No. 3,172,892.

A particular PIBSA polyamine derivative surfactant that has been found to be useful in the process of this invention is one wherein R, and R₂ taken together to form an alkyl succinic radical and wherein the surfactant is a compound having the general formula: wherein m is an integer generally ranging of about 10-60 and more preferably 40, thereby giving said preferred polyamine derivative a molecular weight of about 2000. This surfactant will generally comprise from about 0.2 to 10 weight % of the exterior phase of the emulsion, preferably from about 0.5 to 5 weight % and still more preferably from about 1-3 weight %.

As hereinbefore stated, the external phase of the emulsion must contain an agent capable of transferring the uranium from the aqueous feed, through the oily external phase to the interior phase. Transfer agents found suitable for transferring cationic uranium species containing hexavalent uranium (i.e. UO₂²⁺) through the external phase to the internal phase include a mixture of oil soluble dialkyl esters of phosphoric acid and trialkyl-phosphine oxide. In particular, a mixture of di(2-ethylhexyl) phosphoric acid (D2EHPA) and trioctylphosphine oxide (TOPO) are preferred for transporting uranyl (UO₂²⁺) through the external phase of the emulsion. This mixture will not transfer uranium species wherein uranium exists in the +4 valence U(IV) state. In general, the transfer agent will comprise from between about 1-30 wt. % of the exterior phase of the emulsion, preferably from about 2-18 wt. % and most preferably from about 2-6 wt. %. When the transfer agent comprises a combination of D2EHPA and TOPO they will be in said exterior phase in a molar ratio ranging from about 1/1 to 10/1, preferably from 2/1 to 8/1 and, more preferably from about 2/1 to 7/1 of D2EHPA/TOPO.

As hereinbefore stated, the interior phase of the emulsion will be an aqueous acid solution containing a reagent capable of changing the valence state of the uranium transferred through the oily, external phase to trap the uranium being removed from the aqueous feed where it is in the +6 valence state. This interior phase will be an aqueous acid solution containing a reducing agent to reduce the uranium to a +4 valence state. There should be enough reducing agent present in the internal phase to reduce the uranium ion transported therein. Illustrative, but non-limiting examples of suitable reducing agents include acid solutions of ferrous or chromous ions such as an aqueous solution of ferrous sulfate in phosphoric acid wherein the concentration of the ferrous ion ranges from about 8-50 grams per liter, preferably from 10 to 40 g/liter and wherein the concentration of the phosphoric acid ranges from about 3-12 moles/liter and more preferably from about 5-8 moles/liter. The following reaction is believed to occur when reducing (UO₂²⁺) with acidic ferrous sulfate: It is important that the concentration of phosphoric acid in the internal phase be approximately the same as in the feed in order to avoid excessive swelling and ultimately destruction of the emulsion. As a matter of convenience, the internal phase may be prepared from the WPPA feed by adding iron thereto.

The interior phase will comprise from about 15-80 volume percent of the emulsion, preferably from 30-70 and most preferably from 33-60 volume percent, i.e., the volume ratio of the oily exterior or membrane phase to the aqueous interior phase of the emulsion will range from about 6/1 to 1/4, more preferably from about 2/1 to 1/2, and still more preferably from about 2/1 to 1/1.

The emulsions used in this invention may be prepared by any of the well known methods. Thus, a solution comprising the components of the oily exterior phase is mixed with an aqueous solution which will form the interior phase under high shear conditions attained by the use of high speed stirrers, colloid mills, homogenizers, ultrasonic generators, mixing jets, etc.

As mentioned previously, the excess oxidizing agent can be added to the WPPA feed before it enters the extraction train, or it may be added in stages throughout the extraction sequence, or both. Thus, a portion of the excess may be added to the feed before it is contacted with the emulsion, with the remainder added at one or more points along the extraction train. Alternatively it may all be added to the feed prior to its being contacted with the emulsion or it may all be added to the feed at one or more points of the extraction train.

The invention will be more readily understood by reference to the examples set forth below.

### Examples

### Example 1

In this example, uranyl ion (U0₂ ^{H}) was laboratory batch extracted from an actual sample of central Florida WPPA comprising a 5.2 M solution of H₃P0₄ containing 130 ppm of uranium as UO_{Z}^{++.} The emulsion used to extract the uranium had the following composition:
External phase-2.91 wt. % D2EHPA, 0.88 wt. % TOPO and 5 wt. % of a PIBSA-THAM surfactant of the type disclosed in U.S. Patent No. 4,102,798, (made by reacting 1 mole of PIBSA having a molecular weight of about 1,300 with 1.9 moles of THAM, i.e. tris-hydroxymethyl amino methane) in LOPS:
Interior Phase-a solution of 6M H₃P0₄ containing 30 g/I of ferrous ion; and the volume ratio of exterior to interior phase was 2/1.

The WPPA was filtered through a 1 m cartridge filter to remove the solid gypsum and some organics as solids. The WPPA, 1500 mL, was then added to the resin kettle of 10 cm I.D. fitted with four 1 cm vertical baffles and four evently spaced marine propellers of 5.1 cm diameter. The temperature was increased to and controlled at 60±1°C with external heating.tape and a Thermowatch controller.

The liquid membrane emulsion was prepared in a Waring blender at 10,000 ppm for 4 min. using 333 ml of.membrane and 167 ml of internal aqueous phase. The emulsion, 125 ml, for a feed to emulsion ratio of 12, was added to the resin kettle. Mixing at 600 rpm was then begun and was t=0 for measurement of contact time. In the first run, only 0.068 grams of ammonium persulfate oxidant was added to the kettle which was just enough to ensure that all of the uranium and iron in the WPPA feed were in the +6 and +3 valence state, respectively. This amount of oxidant was enough to give an initial concentration of oxidant in the feed of 0.001 M. For run 2, 0.342 grams of oxidant were added initially (yielded initial conc. of oxidant of 0.005 M) and another 0.342 grams after 10 minutes. In run 3, 0.342 grams were added initially, followed by another 0.342 grams after 20 minutes.

Samples of the dispersion were taken during agitation through a stopcock in the bottom of the resin kettle at various contact times. These samples were allowed to phase separate and aliquots of the raffinates were analyzed for uranium content. At the completion of extraction, a sample emulsion was coalesced to isolate internal phase for uranium analysis by X-ray fluorescence spectroscopy.

The results of these runs are set forth in Table I and illustrate a significant improvement in extraction efficiency using the process of this invention.

### Example 2

In an actual commercial extraction operation, the internal phase of the liquid membrane will contain tetravalent uranium, as U(IV) ion, to a loading in a range of about 6 to 12 g/L. Therefore, extraction of uranium from the WPPA was done with a preloaded emulsion whose internal phase contained 10 g/L of uranium as U⁺⁴. The experimental conditions were the same as in Example 1. The results given in Table II show that no extraction was observed without added oxidant, whereas with added oxidant 47% of the uranium was extracted after 25 minutes contact time. These results demonstrate the significant and surprising improvement provided by the addition of oxidant during LM extraction of uranium.

### Example 3

More related to commercial practices, extraction was also carried out in a continuous contacting system comprising one extraction stage which contained five cocurrent, cascading mixing compartments. Each compartment was a cube of one liter capacity containing a marine propeller mixer. Pretreated WPPA and fresh LM emulsion were fed into the first compartment wherein a dispersion of LM emulsion in the continuous WPPA phase was formed by the shear of the marine propeller-stirrer contained in each compartment. The resultant dispersion cascaded through each successive compartment by overflow after a finite contacting period. Finally, the dispersion overflowed from the last compartment into a settler to allow disengagement and separation of the loaded LM emulsion from the WPPA raffinate phase.

Commercial WPPA was oxidized in polyethylene lined, 55 gal (250 I) drums with hydrogen peroxide and pumped through a 1 m polypropylene cartridge in line filter to a 3 I vessel. This vessel was a preheater which increased the temperature of the pretreated WPPA to 60-70⁰C. The acid was then fed via a peristaltic pump (all fluids were transferred with peristaltic pumps) to the continuous contacting system described above.

The detailed conditions of the experiments are given in Table III.

Samples of raffinate from each mixing compartment were analyzed for uranium content by inductively coupled ion plasma emission spectroscopy.

As seen from the results presented in Table III, a similar improvement in extraction of uranium from WPPA was obtained by the addition of oxidant to WPPA feed during extraction. In this case, a 2.5 M ammonium persulfate solution was added to the fourth mixing compartment at a flow rate of 0.2 ml/min. In Run 5, with no added oxidant, the extraction efficiency at 50 min. contact time was 63%, whereas, with added oxidant in Run 6, the extraction efficiency was 68%. This significant improvement was corraborated by the replicate experiment Run 7.

## Claims

1. An emulsion process for recovering uranium from a WPPA (wet process phosphoric acid) feed solution wherein the uranium ions initially are oxidised by adding an oxidising agent to said feed solution in order to ensure that all uranium is present in the hexavalent form, said process comprising:
(a) contacting said WPPA feed with a water-in-oil emulsion comprising (i) an aqueous interior phase dispersed in (ii) an oily exterior phase immiscible with both said interior phase and said feed, said interior phase comprising an acid solution containing a reducing agent and said exterior phase comprising a surfactant-containing hydrocarbon solution of D2EHPA (di-2-ethylhexyl phosphoric acid) and TOPO (trioctyl phosphine oxide) which transfer the uranyl ion from the WPPA feed to the interior phase of the emulsion wherein said hexavalent uranium ion is reduced to tetravalent uranium ion to form a uranium-rich emulsion;
(b) separating the 'uranium-rich emulsion from the WPPA feed; and
(c) recovering the uranium from the emulsion, characterised in that an oxidising agent is added to the WPPA solution before and/or while the feed is contacted with the emulsion in a quantity in excess of that needed to ensure initially that the uranium in the feed is in the hexavalent state and in a quantity to ensure that any iron in the feed is in the trivalent state.

2. A process according to Claim 1 wherein said interior phase acid solution comprises phosphoric acid and wherein said interior phase comprises from about 15-80 volume percent of said emulsion.

3. A process according to Claim 2 wherein said phosphoric acid solution in said interior phase is at a concentration of from 3-12 moles per litre.

4. A process according to either of Claims 2 and 3 wherein the concentration of said phosphoric acid solution in said interior phase is substantially the same as the concentration of phosphoric acid in said WPPA solution.

5. A process according to any one of the preceding claims wherein said surfactant is a polyamine derivative of polyisobutylene succinic anhydride.

6. A process according to Claim 5 wherein said polyamine derivative of polyisobutylene succinic anhydride has the general formula: wherein R₁, R₂, R₃, R₄, R₅, R₆, and R₇ and Y are the same or different and are hydrogen, c₁ to C₂₀ alkyl, C₆ to C₂₀ aryl, C₇ to C₂₀ alkaryl radicals or substituted derivatives thereof; and x is an integer of from 1 to 100.

7. A process according to Claim 6 wherein R₃ to R₇ are hydrogen and x varies from 3 to 20.

8. A process according to any one of the preceding claims wherein said feed/emulsion contacting is carried out in a plurality of contacting zones.

9. A process according to any one of the preceding claims wherein said oxidising agent is added to said feed after it has initially contacted said emulsion.

## Patentansprüche

1. Emulsionsverfahren zur Gewinnung von Uran aus einer WPPA (Naßverfahren-Phosphorsäure) Einsatzlösung, bei dem die Uranionen Am Anfang durch Zusatz eines Oxydationsmittels zu der Einsatzlösung oxydiert werden, um sicherzustellen, daß alles vorhandenes Uran in der sechswertigen Form vorliegt, und bei dem:
(a) das WPPA-Einsatzprodukt mit einer Wasser-in-Öl-Emulsion kontaktiert wird, die (i) eine wässrige innere Phase aufweist, die in (ii) einer öligen äußeren Phase dispergiert ist, die sowohl mit der inneren Phase als auch mit dem Einsatzprodukt nicht mischbar ist, wobei die innere Phase eine Säurelösung aufweist, die ein Reduktionsmittel enthält, und die äußere Phase eine tensidhaltige Kohlenwasserstofflösung von D2EHPA (Di-2-ethylhexylphosphorsäure) und TOPO (Trioctylphosphinoxid) aufweist, die die Uranylionen aus dem WPPA-Einsatzprodukt in die innere Phase der Emulsion transportieren, wo das sechswertige Uranion zu vierwertigem Uranion unter Bildung einer an Uran reichen Emulsion reduziert wird,
(b) die an Uran reiche Emulsion vom WPPA-Einsatzprodukt getrennt wird und
(c) das Uran aus der Emulsion gewonnen wird, dadurch gekennzeichnet, daß der WPPA-Lösung, bevor und/oder während das Einsatzprodukt mit der Emulsion kontaktiert wird, ein Oxydationsmittel in einer Menge im Überschuß gegenüber der, die zur anfänglichen Sicherstellung, daß das Uran im Einsatzprodukt sich im sechswertigen Zustand befindet, erforderlich ist, und in einer Menge zugesetzt wird, daß sichergestellt ist, daß jegliches im Einsatzmaterial vorhandenes Eisen im dreiwertigen Zustand vorliegt.

2. Verfahren nach Anspruch 1, dadurch gekennzeichnet, daß die Säurelösung der inneren Phase Phosphorsäure enthält und daß die innere Phase etwa 15 bis 80 Vol% der Emulsion ausmacht.

3. Verfahren nach Anspruch 2, dadurch gekennzeichnet, daß die Phosphorsäurelösung der inneren Phase eine Konzentration von 3 bis 12 Mol je Liter aufweist.

4. Verfahren nach Anspruch 2 oder 3, dadurch gekennzeichnet, daß die Konzentration der Phosphorsäurelösung in der inneren Phase im wesentlichen die gleiche ist wie die Konzentration der Phosphorsäure in der WPPA-Lösung.

5. Verfahren nach einem der vorangehenden Ansprüche, dadurch gekennzeichnet, daß das Tensid ein Polyaminderivat von Polyisobutylenbernsteinsäureanhydrid ist.

6. Verfahren nach Anspruch 5, dadurch gekennzeichnet, daß das Polyaminderivat von Polyisobutylenbernsteinsäureanhydrid die allgemeine Formel: besitzt, in der R" R₂, R₃, R₄, R₅, R₆ und R₇ und Y gleich oder verschieden sind und Wasserstoff, C₁―C₂₀-Alkyl-C₆―C₂₀-Ary)-, C₇―C₂₀-Alkarylreste oder substituierte Derivate derselben sind und x eine Zahl von 1 bis 100 ist.

7. Verfahren nach Anspruch 6, dadurch gekennzeichnet, daß R₃ bis R₇ Wasserstoff sind und x von 3 bis 20 variiert.

8. Verfahren nach einem der vorangehenden Ansprüche, dadurch gekennzeichnet, daß das Einsatzprodukt/Emulsion-Kontaktieren in einer Vielzahl von Kontaktierzonen durchgeführt wird.

9. Verfahren nach einem der vorangehenden Ansprüche, dadurch gekennzeichnet, daß das Oxydationsmittel dem Einsatzprodukt zugegeben wird, nachdem der Kontakt des Einsatzproduktes mit der Emulsion begonnen hat.

## Revendications

1. Procédé en émulsion pour récupérer l'uranium d'une solution de charge d'acide phosphorique obtenu par voie humide, procédé dans lequel on oxyde initialement les ions uranium en ajoutant un oxydant à ladite solution de charge pour faire en sorte que la totalité de l'uranium soit présent sous forme hexavalente, ledit procédé consistant:
(a) à mettre en contact ladite charge d'acide phosphorique avec une émulsion du type eau dans huile comprenant (i) une phase intérieure aqueuse dispersée dans (ii) une phase extérieure huileuse non-miscible tant à ladite phase intérieure qu'à ladite charge, ladite phase intérieure comprenant une solution dans un acide contenant un réducteur, et ladite phase extérieure comprenant une solution, dans un hydrocarbure contenant un tensio-actif, de D2EHPA (acide di-2-éthylhexylphosphorique) et de TOPO (oxyde de trioctylphosphine), qui transfèrent l'ion uranyle de la charge d'action phosphorique à la phase intérieure de l'émulsion, dans laquelle ledit ion uranium hexavalent est réduit en ion uranium tétravalent pour former une émulsion riche en uranium;
(b) à séparer l'émulsion riche en uranium de la charge d'acide phosphorique obtenu par voie humide, et
(c) à récupérer l'uranium de l'émulsion, caractérisé en ce qu'on ajoute à la solution d'acide phosphorique avant et/ou pendant que la charge est en contact avec la solution, un oxydant introduit en une quantité supérieure à la quantité nécessaire pour faire initialement en sorte que l'uranium se trouvant dans la charge se présente à l'état hexavalent et en une quantité suffisante pour que la totalité du fer éventuellement présent dans la charge se trouve à l'état trivalent.

2. Procédé selon la revendication 1, dans lequel ladite solution d'un acide dans la phase intérieure comprend de l'acide phosphorique, et dans lequel ladite phase intérieure compte pour environ 15-80% en volume de ladite émulsion.

3. Procédé selon la revendication 2, caractérisé en ce que la solution d'acide phosphorique dans ladite phase intérieure se présente à une concentration de 3 à 12 moles par litre.

4. Procédé selon l'une ou l'autre des revendications 2 ou 3, dans lequel la concentration de la solution d'acide phosphorique dans ladite phase intérieure est pratiquement la même que la concentration de l'acide phosphorique dans ladite solution d'acide phosphorique obtenu par voie humide.

5. Procédé selon l'une quelconque des revendications 1 à 4, dans lequel ledit tensio-actif est un dérivé polyaminique de l'anhydride polyisobutylènesuccinique.

6. Procédé selon la revendication 5, dans lequel ledit dérivé polyaminique de l'anhydride polyisobutylènesuccinique a la forme générale dans laquelle R₁, R₂, R₃, R₄, Rₛ, R₆ et R₇ et Y sont identiques ou différents et sont chacun l'hydrogène, un radical alkyle en Ci à C₂ₒ, aryle en C₆ à C₂₀, alcaryle en C₇ à C₂₀, ou leurs dérivés substitués; et x est un entier de 1 à 100.

7. Procédé selon la revendication 6, dans lequel R₃ à R₇ sont chacun l'hydrogène, et x varie de 3 à 20.

8. Procédé selon l'une quelconque des revendications 1 à 7, dans lequel ladite mise en. contact de la charge et de l'émulsion s'effectue dans plusieurs zones de contact.

9. Procédé selon l'une quelconque des revendications 1 à 8, dans lequel ledit oxydant est ajouté à ladite charge après la mise en contact initiale de cette charge avec ladite émulsion.
